

## UNITED STATES PATENT OFFICE

GUSTAVE LANDT AND HUBERT LEOPOLD BECHER, OF TRENTON, NEW JERSEY, AS  
SIGNORS TO THE AGASOTE MILLBOARD COMPANY, OF FANWOOD ROAD, NEW  
JERSEY, A CORPORATION OF NEW JERSEY

## PULP BOARD

No Drawing.

Application filed August 13, 1924. Serial No. 731,871.

Our invention relates to pulp board and comprises, broadly speaking, pulp board provided with a binder of Montan wax. A board embodying our invention may be made of any of the usual paper pulps, either rag or wood fibre, or may be made of straw, bagasse or other suitable material and may be produced in laminated or homogeneous form. We have obtained our best results with molded pulp board which is made by running paper pulp, wood pulp, or the like into a mold and, by means of pressure, removing the majority of the water (see for instance United States Letters Patent No. 971,936 dated October 4, 1910, and No. 1,272,566 dated July 16, 1918) and subsequently drying out the remainder of the water by the application of heat. The wax may be added to the fibre either before or after the latter has been shaped into a board. For instance the board may be dipped into the melted Montan wax for a sufficient length of time to enable it to absorb a suitable proportion of such wax; or the fibre and the wax, the latter in the form of an emulsion, may be mixed in the beater before molding or laying up the board, although a board made in this manner may not possess as high a degree of tensile or transverse strength as does a board made by the dipping process. We may also dip the dried board into a solution of the wax, thereafter driving out the solvent by heat or otherwise. We have, however, found that by far the best results are obtained by adding the Montan wax in comminuted form to the beater while the pulp is being beaten therein. For this purpose it is advisable to grind the Montan wax dry in a ball mill, as fine as possible and then to moisten it with water and thereafter to complete the grinding in the same mill. The wet ground Montan wax will more readily mix with pulp in the beater as it does not tend to rise to, and float upon, the surface of the water as it would do if added in the form of a dry powder. By adding the Montan wax to the fibre in comminuted form we obtain a more equal distribution thereof throughout the entire sheet and are enabled to fill up all the spaces between the fibres, thus obtaining a more compact and

waterproof board, having a better surface, and absorbing less paint when the surface is painted. We can moreover, by this specific method, mix more Montan wax with the fibre without having the same squeezed out during the compressing process and thus obtain a board of greater tensile strength. The comminuted Montan wax seems to give results far superior to those obtained by the use of the emulsified wax, probably because the former is unchanged (unemulsified). 55 60

The proportion of Montan wax, by weight, to the weight of fibre in the final product is preferably from 30% to 50%, the exact percentage depending upon the use to which the board is to be put; the greater the proportion of Montan wax within these limits, the more waterproof will be the finish board and the higher its tensile strength, other things being equal; on the other hand, the higher the compression to which the saturated board is to be subjected, the smaller would have to be the percentage of Montan wax used. Of course, no such high percentage of Montan wax should be used as would result merely 65 70 75 in the squeezing out of a large amount of it during the compressing process.

A board made as above described has high tensile and transverse strength and a high degree of hardness. A board thus produced is also substantially waterproof and highly di-electric. A stiff board made as above described may readily be bent to any suitable form, or embossed, after the same has been rendered plastic by heating it slightly above 80 85 the fusion point of the wax. On the other hand, it will not be injured by exposure to the sun when used as roofing or siding for buildings.

In spite of its high tensile and transverse strength, the material may be easily toolled and does not dull tools to the same extent as will such materials, of equal hardness, which are known to us and which are made of pulp treated with other binders. The material 90 95 has very good wearing qualities and can, therefore, be used for various purposes in which such qualities are important, for instance, as tread material for protecting steps.

We do not claim the use of so small, or so 100

large, a proportion of Montan wax to fibre that the advantages hereinabove set forth are not obtained. We realize, however, that the use of somewhat less and somewhat more than the optimum proportions of 30 to 50 parts by weight of Montan wax to 100 parts by weight of fibre may result in obtaining the advantages hereinabove stated to a lesser degree and to that extent the use of such proportions would be within the spirit of our invention and the equivalent of the proportions specified in our claims.

10 A board made as hereinabove described, to which other ingredients have been added without changing its essential characteristics, would fall within the scope of our invention.

15 We claim:

1. Molded pulp board comprising a compressed mixture of from 30 to 50 parts of Montan wax, by weight, to 100 parts of fibre.

20 2. An article of the character described consisting of fiber board impregnated for a substantial depth with a waxy material which is hard and brittle at high atmospheric temperatures but is sufficiently fluid at 275° F. to be forced into said fiber board.

25 3. An article of the character described consisting of fiber board rendered substantially impervious to moisture by having the pores and cells thereof for a substantial depth filled with a hard waterproof waxy material which will not soften at temperatures below 140° F.

30 4. An article of the character described consisting of fiber board impregnated for a substantial depth with a composition in which Montan wax predominates.

35 5. An article of the character described consisting of fiber board impregnated for a substantial depth with Montan wax.

40 6. An article of the character described consisting of fiber board carrying in the microscopic pores and cells thereof a waterproof waxy material which remains hard at temperatures below 140° F. but becomes sufficiently fluid at 275° F. to be forced into said pores and cells.

45 7. The process of improving the characteristics of fiber board which consists in impregnating it for a substantial depth with a melted waxy material which is hard and brittle at high atmospheric temperatures but becomes sufficiently fluid at 275° F. to penetrate into the microscopic pores and cells of fiber board, and subsequently allowing the fiber board so treated to cool sufficiently to cause said material to harden therein.

GUSTAVE LANDT.  
HUBERT LEOPOLD BECHER.